

## UNITED STATES PATENT OFFICE

2,192,228

## DELMING OF HIDES AND SKINS

William H. Hill, Stamford, Conn., assignor to  
American Cyanamid Company, New York, N. Y.,  
a corporation of Maine

No Drawing. Application May 26, 1939,  
Serial No. 275,914

2 Claims. (Cl. 149—3)

This invention relates to the deliming of hides and skins by the use of hydroxy aminotriazines as deliming agents.

I have found that aminotriazines containing 5 one or two hydroxy groups are very satisfactory deliming agents for removing lime from hides and skins during their conversion into leather. When used for this purpose they are somewhat slower than such commercially used deliming agents as 10 lactic acid and ammonium salts, but they are much milder in action and will not injure the skin even when contacted therewith for long periods of time.

The hydroxy aminotriazines are the members 15 of the group consisting of ammeline, which is 1-hydroxy-3,5-diamino-2,4,6-triazine, ammelide, which is 1-amino-3,5-dihydroxy-2,4,6-triazine and condensation products containing two triazine nuclei linked by an imino group and having 20 at least one amino group and one hydroxy group attached thereto. They are obtained as by-products in the production of melamine by the heat conversion of dicyandiamide, or directly by the condensation of dicyandiamide or biguanide salts 25 with urea. The polycyclic compounds containing two triazine nuclei are found among the by-products obtained when dicyandiamide is heated with sodium or potassium carbonate for the production of melamine.

30 All of the hydroxy aminotriazines of the above described class are white crystalline solids which are only slightly soluble in water, but which form water-soluble calcium salts. I have found, however, that ammeline possesses the most desirable deliming characteristics of any member 35 of this group and my preferred deliming agents contain this material, either alone or in admixture with ammelide and hydroxy aminotriazines of higher molecular weight. Since considerable 40 quantities of ammeline are present in the crude mixture obtained as a by-product in the production of melamine from dicyandiamide, the use of these crude mixtures as deliming agents is also

included in this preferred embodiment of the invention.

The hydroxy aminotriazines are particularly well suited for use in deliming processes employing a large excess of deliming agent as where 5 complete deliming of the hide or skin is desired but without damage to the grain. They are therefore especially well suited for the manufacture of light leathers of high quality, such as up-holstery leather, embossed leather and the like. 10

The invention will be illustrated in greater detail by the following specific example, to which, however, it is not limited.

## Example

15 A dried goat skin was soaked in water for 24 hours and was then immersed in a lime bath containing an excess of lime for seven days. It was then unhaired, washed, drained and weighed.

The unhaired skin was placed in a paddle 20 washer containing 400% of its weight of water and 10% of ammeline and washed overnight with continuous agitation by the paddle. At the end of this period the pH of the solution was 7.7 and that of the skin was 7.0 as indicated by brom 25 thymol blue. Both skin and solution were colorless to phenolphthalein and the skin was thoroughly delimed.

The 10% of ammeline used was a considerable 30 excess, as was shown by the presence of undissolved crystals of ammeline in the bottom of the bath. However there was no deposition of material on the skin and the grain was clear and firm, indicating that even large amounts of the deliming agent were not injurious to the leather. 35

What I claim is:

1. A method of deliming hides and skins which comprises immersing them in an aqueous dispersion containing a hydroxy aminotriazine.
2. A method of deliming hides and skins which 40 comprises immersing them in an aqueous dispersion containing ammeline.

WILLIAM H. HILL.